

## UNITED STATES PATENT OFFICE

2,232,922

## MAGNESIUM BASE ALLOY

John C. McDonald, Midland, Mich., assignor to  
The Dow Chemical Company, Midland, Mich.,  
a corporation of Michigan

No Drawing. Application January 31, 1940,  
Serial No. 316,514

3 Claims. (Cl. 75—168)

The invention relates to magnesium base alloys, and more particularly concerns an alloy of this nature having a high degree of formability associated with other desirable physical properties such as excellent yield and tensile strengths.

Magnesium alloys are being widely used in the various structural and mechanical arts where a light weight metal is highly desirable, such as for use in making castings, forgings, and the like. However, the use of these alloys in the rolled form to make sheet metal articles requiring forming operations, such as bending, drawing and the like, has not progressed as rapidly due to the fact that in general alloys of good formability permitting relatively sharp bends to be made without the article developing external cracks usually have inferior strength characteristics.

It is accordingly the principal object of the invention to provide a magnesium base alloy which can be made into rolled sheet or the like possessing a sufficient degree of ductility or formability to be sharply bent, drawn, or otherwise shaped while having good tensile and yield strengths.

Other objects and advantages will be apparent as the description of the invention proceeds.

from about 1 to 5 per cent of silver and from 0.1 to 0.3 per cent of calcium. The specific proportion of each alloying metal and the total amount of alloying metals to be added to the new alloy depends upon the use for which the alloy is intended. For example, where good ductility or formability associated with excellent yield and tensile strengths is of principal importance, the alloy should preferably contain from about 4 to 8 per cent of silver and from 0.1 to 0.2 per cent of calcium. While in those instances where exceptionally high yield and tensile strengths are more important, the alloy should contain from 10 to 15 per cent of silver and from 0.1 to 0.3 per cent of calcium.

The following table lists some of the properties of rolled sheet metal made from my new ternary alloy and compares these properties with those of rolled sheet made from related binary alloys. A comparison of the properties illustrates the improvement in the strength characteristics of the new alloy over that of the closely related binary alloy. In the table the per cent elongation is to be regarded as a measure of the ductility or formability of the specimen.

Table

| 30 | Nominal composition in percent (magnesium—remainder) |      | Annealed |    |                                | Cold rolled                      |                                | 30     |        |
|----|------------------------------------------------------|------|----------|----|--------------------------------|----------------------------------|--------------------------------|--------|--------|
|    |                                                      |      | Ag       | Ca | Yield strength in lbs./sq. in. | Tensile strength in lbs./sq. in. | Percent elongation in 2 inches |        |        |
| 35 | 0.15                                                 |      | 18,000   |    | 32,000                         |                                  | 17                             | 29,000 | 35,000 |
|    | 2                                                    | 0.15 | 19,000   |    | 32,000                         |                                  | 15                             | 28,000 | 35,000 |
|    | 2                                                    | 0.15 | 19,000   |    | 32,000                         |                                  | 17                             | 35,000 | 40,000 |
|    | 4                                                    |      | 21,000   |    | 34,000                         |                                  | 20                             | 33,000 | 39,000 |
|    | 4                                                    | 0.15 | 20,000   |    | 35,000                         |                                  | 18                             | 39,000 | 45,000 |
|    | 8                                                    |      | 25,000   |    | 38,000                         |                                  | 16                             | 37,000 | 44,000 |
|    | 8                                                    | 0.15 | 24,000   |    | 38,000                         |                                  | 13                             | 43,000 | 52,000 |
| 40 | 12                                                   |      | 27,000   |    | 42,000                         |                                  | 8                              | 39,000 | 47,000 |
|    | 12                                                   | 0.15 | 27,000   |    | 41,000                         |                                  | 7                              | 44,000 | 53,000 |

45 My invention resides in the discovery that a magnesium base alloy composed of from 0.1 to 20 per cent of silver and from 0.01 to 1 per cent of calcium, the balance being substantially all magnesium is endowed with the afore-mentioned properties. While the properties of good formability or ductility associated with excellent tensile and yield strengths are manifest over the entire range of the composition indicated, I have found that in general the preferred combination of 50 properties is obtained when the alloy contains

45 The properties listed in the above table under the section headed by the term "annealed" were obtained by first rolling the alloys at a temperature of 600° F. and thereafter annealing them at various temperatures, in the temperature range from 400° to 600° F. The properties selected 50 for the table were those of the annealed specimens which exhibited the maximum elongation. Properties listed in the above table under the section headed "cold rolled" were obtained by subjecting specimens of the alloy which had been 55

hot rolled at a temperature of 600° F. to additional rolling in the cold state to bring about a total reduction of from 2 to 10 per cent. The properties selected for the table were those of the cold rolled specimens which showed the greatest tensile and yield strength while having at least 1 per cent elongation in 2 inches.

By comparison of the properties listed in the above table, it will be observed that the combined properties of my new ternary alloy are superior to those of the binary alloys having similar percentages of alloying ingredients. For example, it will be noted that the alloys containing lower percentages of alloying ingredients have an excellent elongation coupled with markedly superior strength properties in the cold rolled state. In the higher percentages of alloying ingredients, the strength characteristics of the new alloy in the cold rolled state also show a high degree of improvement. Similar improvement will be noted throughout the range of alloying ingredients indicated.

While the new alloy is most useful in the wrought form, such as sheets, due to its formability characteristics, it may also be suitably used in making castings, forgings, extruded forms and the like. It is further pointed out that my new alloy is amenable to solution and

precipitation heat treatments, which, accordingly, modify its properties.

The new alloy may be compounded in any of the ways known in the art, such as by adding the alloying ingredients to molten magnesium under suitable flux. The flux should be substantially free from magnesium chloride if the calcium content is to be above 0.3 per cent. In those instances where the calcium content is to be less than 0.3 per cent, magnesium chloride may be present in the flux without exerting any deleterious effects, but in this case it is preferable to add the calcium last without too much stirring or agitation in order to prevent the loss of some of the calcium into the flux.

I claim:

1. A magnesium base alloy containing from 0.1 to 20 per cent of silver, from 0.01 to 1 per cent of calcium, the balance being substantially all magnesium.

2. A magnesium base alloy containing from 2 to 8 per cent of silver and from 0.1 to 0.2 per cent of calcium, the balance being magnesium.

3. A magnesium base alloy containing from 8 to 15 per cent of silver and from 0.15 to 0.3 per cent of calcium, the balance being magnesium.

JOHN C. McDONALD.